

No. 856,475.

PATENTED JUNE 11, 1907

## F. VON KÜGELGEN & G. O. SEWARD. PRODUCTION OF CALCIUM ALLOYS.

APPLICATION FILED MAR. 30, 1905.



## INVENTORS

## WITNESSES:

WITNESSES:  
Fred White  
Rene' Pierre

Franz von Kuegelen & George O. Stewart,  
By Attorneys,  
William G. Draper 

# UNITED STATES PATENT OFFICE.

FRANZ VON KÜGELGEN AND GEORGE O. SEWARD, OF HOLCOMBS ROCK,  
VIRGINIA.

## PRODUCTION OF CALCIUM ALLOYS.

No. 856,475.

Specification of Letters Patent.

Patented June 11, 1907.

Application filed March 30, 1905. Serial No. 252,798.

*To all whom it may concern:*

Be it known that we, FRANZ VON KÜGELGEN, a subject of the German Emperor, and GEORGE O. SEWARD, a citizen of the United States, both residing at Holcombs Rock, Bedford county, Virginia, have jointly invented certain new and useful Improvements in the Production of Calcium Alloys, of which the following is a specification.

Our invention relates to the electrolysis of a salt of calcium whereby to produce calcium alloys. The metal to be alloyed with the calcium is fused and serves as the cathode.

According to our invention we may produce an alloy of calcium and zinc by electrolysis of molten calcium chlorid ( $\text{CaCl}_2$ ), using a cathode of molten zinc. Calcium and zinc alloy in almost any proportion. All calcium-zinc alloys except those containing very little zinc are heavy enough to remain at the bottom of the cell where the alloy is unattacked by the chlorin which is liberated at the anode. These calcium-zinc alloys are advantageous for use as reducing agents, for which purpose the zinc is not disadvantageous. It is well known that calcium is a very active reducing agent, but it is expensive and difficult to make. The calcium-zinc alloys are easily made, the apparatus being simple and durable, and the process easily managed, while the cost is low because of the low voltage required. The alloys if containing even as much as ten per cent. zinc are brittle and easily powdered. These alloys promise to have a wide application as reducing agents in place of aluminum or pure calcium.

The accompanying drawing shows in vertical section a suitable form of an electrolytic cell for practicing our process.

Let A designate the cell or vessel, B the dynamo or other source of current, and C the anode, which may be of carbon, graphite or any other suitable substance. The bottom of the cell is filled with molten zinc ( $\text{Zn}$ ) above which floats the electrolyte of fused calcium chlorid ( $\text{CaCl}_2$ ) in which the anode is immersed. Heat may be applied in any suitable way to fuse this salt, the fusion of which maintains the zinc in molten condition because of the lower melting point of the latter.

The fusion may be effected by externally applied heat, as, for example, by means of a gas burner *a* beneath; or it may be effected, and in practice will ordinarily be

maintained after the operation is started, by electric heating due to the resistance of the electrolyte to the passage of the current. The electric circuit is completed by conductors *b b*.

The electrolytic action disengages chlorin at the anode, which may be collected and carried off in any known manner; the calcium passes to the cathode where it alloys with the zinc. When the alloy becomes sufficiently rich in calcium, the alloy should be drawn off by tapping or otherwise and fresh zinc supplied. Or, if a continuous process is not desired, zinc may be added from time to time and the anode raised until as much of the alloy is produced as the vessel will conveniently hold, whereupon the process may be discontinued and the alloy removed.

The vessel A may be of cast iron, in which case it may be the medium through which the negative conductor is put into communication with the zinc cathode, as shown. In such case no portion of the iron vessel should act as a cathode. This may be prevented by water-jacketing the upper portion of the vessel, as shown, *c* being a water-jacket and *d d* the pipes for admitting and conducting away the water. The effect of thus cooling the upper portion of the vessel is that a layer of calcium chlorid is solidified against the cooled surface, as shown at *e*, and protects it. Any other way of confining the cathode to the zinc itself may be adopted.

Our invention is susceptible of modification in both the process and the apparatus for practicing it, as will be well understood.

We claim as our invention:

1. The process which consists in electrolyzing a molten calcium salt in the presence of a cathode of fused zinc whereby is produced an alloy of calcium and zinc.

2. The process which consists in electrolyzing molten calcium chlorid in the presence of a cathode of fused zinc whereby the separated calcium alloys with such metal.

In witness whereof, we have hereunto signed our names in the presence of two subscribing witnesses.

FRANZ VON KÜGELGEN.  
GEORGE O. SEWARD.

Witnesses:

GEO. I. LANCASTER,  
F. VON BIDDER.